

## UNITED STATES PATENT OFFICE.

GEORGE S. BOHART, OF SAN FRANCISCO, CALIFORNIA, ASSIGNOR TO NATIONAL CANNERS ASSOCIATION, OF WASHINGTON, DISTRICT OF COLUMBIA, A CORPORATION OF DELAWARE.

## PROCESS AND PRODUCT FOR PREVENTING DISCOLORATION OF CANNED FOODS.

No Drawing.

Application filed March 13, 1926. Serial No. 94,598.

The invention relates to new and useful improvements in a process for preventing discoloration of canned foods, and is a continuance in part of application Serial No. 5 90,709, filed by me February 25, 1926.

It is a well known fact that in the processing of many canned foods, there are formed sulphur compounds which occasionally react either during processing or subsequent thereto, with tin plate metal containers forming dark colored compounds, which are objectionable in appearance.

The present invention is directed to a process whereby the formation of such dark colored compounds is prevented.

Through a series of experiments of processing foods in tin cans, it has been found that if an insoluble metallic compound, such as zinc oxide or zinc phosphate or a mixture 20 of the two or other insoluble oxides or salts of metals which do not form objectionable colored sulphides, is thoroughly incorporated with the ingredients of a protective coating of lacquer and homogeneously distributed through said lacquer prior to the application of the lacquer to the tin plate, so that said compound becomes a component 25 part of the lacquer, discoloration of the food packed in such cans is avoided. The inner 30 surface of the body and ends should both carry the lacquer to inhibit sulphide discoloration of the cans or contents.

In carrying out the invention, an insoluble metallic compound of the character specified is properly mixed with the ingredients forming the lacquer which is to be coated on the metal. The quantity of zinc oxide, for example, mixed with the lacquer may be varied within such limits as to produce a 40 lacquer on the tin plate carrying quantities of metallic zinc varying from one-one hundredth of a milligram to two milligrams per square inch of lacquered surface.

The following mixtures have proved practical in actual use and are detailed below, it being distinctly understood that this invention is not limited to the specific mixtures or conditions shown:

1. Cumar, 10 parts and zinc oxide, 5 parts.
2. Cumar, 18 parts, gutta-percha, 4 parts, and zinc oxide, 11 parts.
3. Cumar, 18 parts, chicle gum, 4 parts, and zinc oxide, 11 parts.

4. Carnauba wax, 1 part; chicle gum, 1 part and zinc oxide, 1 part.

In making up these mixtures, the cumar, chicle gum, and gutta-percha were dissolved in about five parts by weights of carbon tetrachloride or in some cases a little more. After complete solution, the zinc oxide was stirred in, and the mixture was passed through a paint mill twice in order to grind the zinc oxide finely enough to keep it in suspension. Carbon tetrachloride was then added in sufficient amount to reduce the total 65 solids present (including gums, waxes and zinc oxide) to five per cent. The mixture was applied to the metal of the cans.

When the insoluble metallic compound is incorporated in the lacquer after the manner above described, it becomes permanently embodied in the lacquer and will be held in place on the inside of the container during 70 processing and subsequently thereto.

I have found by actual experience that the lacquers which can be defined as baking lacquers stand up the best and give the most satisfactory results. It is customary to bake the lacquer with the metallic compound therein on the metal adapted to form the inner surface of the can. Where the cans are stacked on end, it has also often been proved in practice that it is not necessary to apply this lacquer bearing the insoluble metallic compound over the entire inner surface of 75 the metal container, but if the ends of the container are thus coated, discoloration is avoided.

Magnesium powder, zinc dust and aluminum powder, either singly or in combination, can be mixed with the lacquer and have been found under certain conditions to well serve the purpose of preventing discoloration, since these metals prevent the formation of objectionably colored compounds. 80 The lacquer may then be prepared in the ordinary way and the sheets coated therewith. These coated sheets may be used in making the entire container, or may be used in making the ends or bodies only of the 85 container.

I claim:

1. The process of preventing the discoloration of canned foods comprising providing a portion of the inner surface of the 100 metal forming the container for the food

- with a holding coating having incorporated therewith and homogeneously distributed therethrough an insoluble metallic substance, or substances, which do not form 5 objectionable colored sulphides.
2. The process of preventing the discoloration of canned foods comprising providing a portion of the inner surface of the metal forming the container for the food 10 with a holding coating having incorporated therewith and homogeneously distributed therethrough an insoluble metallic salt, or salts, which do not form objectionable colored sulphides.
- 15 3. The process of preventing the discoloration of canned foods comprising providing a portion of the inner surface of the metal forming the container for the food with a holding coating having incorporated therewith and homogeneously distributed therethrough an insoluble metallic oxide, or oxides, which do not form objectionable colored sulphides.
- 20 4. The process of preventing the discoloration of canned foods comprising providing a portion of the inner surface of the metal forming the container for the food with a holding coating having incorporated therewith and homogeneously distributed therethrough zinc oxide which does not form 25 objectionable colored sulphides.
- 45 5. The process of preventing the discoloration of canned foods comprising providing a portion of the inner surface of the metal forming the container for the food with a baking lacquer coating having incorporated therewith and homogeneously distributed therethrough an insoluble metallic substance, or substances, which do not form 30 objectionable colored sulphides.
- 40 6. The process of preventing the discoloration of canned foods comprising providing a portion of the inner surface of the metal forming the container for the food 45 with a baking lacquer coating having incorporated therewith and homogeneously distributed therethrough an insoluble metallic salt, or salts, which do not form objectionable colored sulphides.
- 50 7. A can for preventing the discoloration of foods contained therein comprising metallic body and ends, the inner surface of one of which is covered with a holding coating and an insoluble metallic substance or substances homogeneously distributed throughout the coating having the property of forming sulphides which are not of objectionable 55 coloration.
- 60 8. A can comprising metallic body and ends, the inner surface of one of which is covered with a baking lacquer throughout which is homogeneously distributed zinc oxide.
- 65 9. The process of preventing the discoloration of canned foods comprising providing a portion of the inner surface of the metal forming the container for the food with a baking lacquer coating having incorporated therewith and homogeneously distributed therethrough an insoluble metallic oxide or oxides, which do not form 70 objectionable colored sulphides.
- 75 10. The process of preventing the discoloration of canned foods comprising providing a portion of the inner surface of the metal forming the container for the food with a baking lacquer coating having incorporated therewith and homogeneously distributed therethrough zinc oxide which does not form 75 objectionable colored sulphides.
- 80 11. A can closure, one of the surfaces of which is covered with a packing lacquer having zinc oxide distributed therethrough.
- 85 12. A can closure having applied to one surface a resinous coating material in which is incorporated an insoluble metallic substance which does not form objectionable colored sulphides.
- 90 13. The process of preventing the discoloration of canned foods comprising providing the inner surface or a portion thereof, of the metal forming the container for the food, with a lacquer coating having an insoluble metallic compound of such metal or metals forming sulphides which are not dark colored thoroughly incorporated with the ingredients and homogeneously distributed through the lacquer prior to the application of the lacquer to the surface of the metal, so that said compound is permanently embodied in the lacquer and held in place on the inside of the container during processing and subsequent thereto.
- 95 14. The process of preventing the discoloration of canned foods comprising providing the interior surface of the metal forming the container for the food with a holding coating having incorporated therewith and homogeneously distributed therethrough an insoluble metallic substance or substances which do not form 100 objectionable colored sulphides.
- 105 15. The process of preventing the discoloration of canned foods comprising providing the inner surface of the metal forming the container for the food with a holding coating having incorporated therewith and homogeneously distributed therethrough an insoluble metallic salt which does not form 110 objectionable colored sulphides.
- 115 16. The process of preventing the discoloration of canned foods comprising providing the interior surface of the metal forming the container for the food with a holding coating having incorporated therewith and homogeneously distributed therethrough an insoluble metallic oxide which does not form 120 objectionable colored sulphides.
- 125 17. The process of preventing discoloration of canned foods comprising providing the inner surface of the metal forming the 125

- container for the food with a holding coating having zinc oxide incorporated therewith and homogeneously distributed therethrough.
5. 18. A can for the preventing of discoloration of foods contained therein comprising metallic body and ends, the inner surfaces of which are covered with a holding coating and an insoluble metallic substance homogeneously distributed throughout the coating having the property of forming sulphides which are not of objectionable coloration.
19. A can comprising metal body and ends, the inner surface of which is covered with a coating throughout which zinc oxide is homogeneously distributed.
10. 20. A product for application to the interior surfaces of cans to prevent discoloration of the food products therein comprising a coating and an insoluble metallic substance homogeneously distributed throughout the coating having the property of forming sulphides which are not of objectionable coloration.
15. 21. A product for application to the interior surfaces of cans to prevent discoloration of the food products contained therein
- comprising a coating and an insoluble metallic oxide incorporated therein.
22. A coating product for cans comprising a lacquer having zinc oxide distributed therethrough.
23. A tinned receptacle having its interior covered with a resinous material in which is incorporated a metallic compound which does not form objectionable colored sulphides.
24. A tinned receptacle for packing food products having its interior coated with a resinous substance having zinc oxide dispersed therethrough.
25. A tinned receptacle for packing food products having its interior coated with a resinous substance in which is incorporated a material which does not form objectionable colored sulphides.
26. A tinned metallic can for packing food products comprising a body and end pieces, the interior of which is coated with a substance having zinc oxide incorporated therewith.

In testimony whereof I affix my signature.

[L. s.] GEORGE S. BOHART.